

## 1

3,668,000

**ANTI-SOILING POLYESTER TEXTILE MATERIAL**  
Alex S. Forschirm, Lake Hiawatha, and Louis E. Trepasso,  
Westfield, N.J., assignors to Celanese Corporation, New

York, N.Y.

No Drawing. Continuation-in-part of application Ser. No.  
845,039, July 25, 1969. This application Apr. 2, 1970,  
Ser. No. 22,140

Int. Cl. B23b 27/06; D06m 15/04

U.S. Cl. 117—138.8 F

3 Claims

### ABSTRACT OF THE DISCLOSURE

There is provided a method of preventing wet-soil redeposition and improving the stain-release characteristics of textile materials comprised of from about 20 to about 100 percent (by weight) of polyester comprising the step of incorporating into said textile material from about 0.0001 to about 10 percent (by weight of polyester fiber in said textile material) of hydroxypropyl methyl cellulose prior to the time said textile material is laundered.

This is a continuation-in-part of application Ser. No. 845,039 filed July 25, 1969 and now abandoned.

Wet-soil-redeposition has been recognized as a major source of soiling for a number of years. In simplified terms this phenomenon is the spreading-out of localized soil over the entire area of a textile product being cleaned or as sometimes happens the transfer of soil from a heavily soiled product onto a lightly soiled product during cleaning. There are certain generally accepted theories as to how redeposition occurs during laundering.

When soiled articles are placed in a laundry machine with water and detergent, theoretically the soil is removed from the fabrics and dispersed by the detergent. The degree of soil removal from the fabric is dependent upon many factors, including water temperature, type and amount of soil, type and amount of detergent, and the chemical composition of the textile fibers being laundered. If the detergent present in the wash water is not functioning with the proper degree of efficiency, all of the soil will not be held in dispersion. In practical terms, this results in what can be described as a three-way equilibrium between soil remaining on the surface of the fabric, soil dispersed by the detergent and soil which is mechanically suspended in the wash water by the agitation forces of the laundry equipment. The laundry machine represents a dynamic system; this results in a general re-distribution of the soil not held in dispersion over the surfaces of the fabric in the wash load.

In an effort to overcome wet-soil-redeposition, and especially wet-soil-redeposition on cotton fiber containing fabrics, the detergent industry has incorporated certain additives such as for instance sodiumcarboxymethyl cellulose. Redeposition of soil in the detergent process consists essentially of the deposition of dispersed particulate soil which may be considered to be in a colloidal state onto a fabric in a detergent liquor. Colloidal properties arise from a large value for the ratio of surface area to mass, although this does not, of course, extend to

## 2

molecular dimensions. Therefore, it is reasonable to consider that the fabric, with its very irregular surface and consequently large surface area, should also exhibit colloidal behavior in a detergent bath. On the basis of the above assumption, soil redeposition may be considered as being equivalent to the coagulation of the colloidal dispersion and the colloidal stability therefore should be applicable. The system consisting of dispersed soil and fabric detergent liquor may be treated as a colloidal system. Colloid stability or soil redeposition is governed by the result of three component forces: (1) an electrical force which may be either attractive or repulsive and that is due to a double layer interaction; (2) an attractive force that arises from the dispersion forces, and (3) a non-electrical repulsive force that is due to a non-electrical interaction of the surface adsorption layers of the particles. The ionogenic whiteness retention additives such as the sodium salt of carboxymethyl cellulose functions primarily by increasing the electrical repulsive force as a result of being adsorbed on soil and/or fabric. Carboxymethyl cellulose however, has not been proved to be suitable for incorporation into heavy duty liquid detergent mixtures, nor has carboxymethyl cellulose completely solved the soil redeposition problem in polyester fiber containing fabrics.

It is thus an object of this invention to provide a method of preventing wet-soil redeposition and improving the stain release characteristics of polyester textile materials. In accordance with this invention, there is provided a method of preventing wet-soil redeposition and improving the stain-release characteristics of textile materials comprised of from about 20 to about 100 percent (by weight) of polyester comprising the step of incorporating into said textile material from about 0.0001 to about 10 percent (by weight of polyester fiber in said textile material) of hydroxypropyl methyl cellulose prior to the time said textile material is laundered.

In the process of this invention, from about 0.0001 to about 10 percent (by weight of polyester fiber in the textile material) of hydroxypropyl methyl cellulose is incorporated into a polyester textile material, although it is preferred to incorporate from about 0.1 to about 2 percent of hydroxypropyl methyl cellulose into said textile material, and it is most preferred to incorporate from about 0.5 to about 1.5 percent of said additive into the textile material. The polyester textile material used in the process of this invention is comprised of from about 20 to about 100 percent (by weight) of linear synthetic polyester, i.e., polyester prepared from terephthalic acid or its dialkyl ester and a polymethylene glycol of the formula  $\text{HO}(\text{CH}_2)_n\text{OH}$  wherein  $n$  is an integer of from 2 to about 8. It is preferred that said textile material be comprised of at least 50 weight percent of said polyester and that  $n$  be from 2 to 4. In the most preferred embodiment, when  $n$  is 2, poly(ethylene terephthalate) is used in the process of this invention.

The hydroxypropyl methyl cellulose may be incorporated into said textile material by methods well known to the art. Thus, e.g., it can be added to fiber by running fiber through a bath comprised of said additive, by padding said additive onto fiber or fabric, by spraying it onto

the textile material during beaming, by putting it on with a lube wheel, etc.

This process of this invention is applicable to any textile material such as, e.g., fiber, yarn, fabric, etc. It is preferred to work with fiber.

In the process of this invention, hydroxypropyl methyl cellulose is applied to the textile material prior to the time said textile material is laundered. Unlike other various water soluble polymers, it affords durable antisoil protection to the treated textile material.

The basic structure for hydroxypropyl methyl cellulose may be shown according to the following formula wherein  $n$  is a finite number:



Hydroxypropyl methyl cellulose may be prepared by swelling cotton linters or wood pulp with a caustic soda solution to produce alkali cellulose which is treated with methyl chloride and propylene oxide yielding cellulose ether with varying ratios of propylene glycol ether substitution to methoxyl substitution on the anhydroglucosidic units.

In order to illustrate applicants' invention, the below mentioned example is presented but is not to be deemed limitative thereof. Unless otherwise stated, all parts are by weight and all temperatures are in degrees centigrade.

**EXAMPLE 1**

100 percent polyester fabrics were submersed in 2 percent aqueous solutions of various water soluble polymers, the fabrics were then dried in an air circulating oven at 80 degrees centigrade for 30 minutes, and laundered. After each laundering the antisoil properties of the fabrics were tested.

The following water soluble polymers were used:

**polyacrylic acid**  
**polyvinyl alcohol**  
**polyethylene oxide**  
**ethylene-maleic anhydride copolymers**  
**methyl vinyl ether-maleic anhydride copolymer**  
**poly acrylamide**  
**hydroxyethyl ethyl cellulose**

Each of these materials afforded some degree of antisoil protection to the treated fabric but, in each instance, said protection was completely lost after only one laundering.

In the manner described above, a 100 percent polyester fabric was treated with a 2 percent solution of hydroxypropyl methyl cellulose. After five launderings, the fabric treated with hydroxypropyl methyl cellulose still exhibited antisoiling properties. It is believed by applicants that this substantivity for the surface of the polyester fiber is a function of the fact that hydroxypropyl methyl cellulose exhibits an inverse solubility effect—the higher the tem-

perature, the lower the solubility; and it is thus believed that other wet-soil-redeposition agents (such as, e.g., polyhydroxyethylmethacrylate) which exhibit an inverse solubility effect should work well as wet soil redeposition agents and afford protection to the treated textile material through many launderings.

Other synthetic textile materials were treated with hydroxypropyl methyl cellulose to determine whether it would impart wet-soil-redeposition characteristics to them.

10 It was found that treated fabric comprised of nylon, treated fabric comprised of acrylic, and treated fabric comprised of cellulose triacetate had antisoil properties imparted to them by the additive of this invention and that

25 said antisoil properties were still exhibited by said fabrics after five launderings.

30 Although the above examples and descriptions of this invention have been very specifically illustrated, many other modifications will suggest themselves to those skilled in the art upon a reading of this disclosure. These are intended to be comprehended within the scope of this invention.

What is claimed is:

35 1. A method of preventing wet-soil redeposition and  
improving the stain-release characteristics of polyester  
fiber comprising the step of incorporating into said fiber  
from about 0.0001 to about 10 weight percent of hydroxy-  
propyl methyl cellulose prior to the time said fiber is  
laundered.

10 2. The process of claim 1, wherein from about 0.1 to about 2 weight percent of hydroxypropyl methyl cellulose is incorporated into said fiber.

3. The process of claim 2, wherein said polyester is poly(ethylene terephthalate).

## References Cited

UNITED STATES PATENTS

|           |         |                        |             |
|-----------|---------|------------------------|-------------|
| 3,391,019 | 7/1968  | Owen et al. -----      | 117-166 X   |
| 3,240,553 | 3/1966  | Paul -----             | 117-139.5   |
| 2,301,509 | 11/1942 | Bock et al. -----      | 117-139.5   |
| 2,663,989 | 12/1953 | Schlatter et al. ----- | 117-139.5   |
| 3,068,120 | 12/1962 | Jacobson et al. -----  | 117-139.5 X |
| 2,979,157 | 4/1961  | Clark -----            | 117-166 X   |
| 3,252,826 | 5/1966  | Salzinger -----        | 117-166 X   |
| 3,226,250 | 12/1965 | Reithel -----          | 117-166 X   |
| 3,455,714 | 7/1969  | Bishop et al. -----    | 117-166 X   |

WILLIAM D. MARTIN, Primary Examiner

80 S. L. CHILDS, Assistant Examiner

U.S. Cl. X.R.

117—138.8 N, 144, 166